

Patented Dec. 21, 1926.

1,611,169

## UNITED STATES PATENT OFFICE.

CAMILLE DREYFUS, OF BASEL, SWITZERLAND, AND GEORGE W. MILES, OF SANDWICH, MASSACHUSETTS, ASSIGNEES TO THE AMERICAN CELLULOSE & CHEMICAL MFG. CO., LTD., OF NEW YORK, N. Y., A CORPORATION OF DELAWARE.

### COMPOSITION OF CELLULOSE ETHERS AND ESTERS WITH HYDROSCOPIC SUBSTANCES AND THE METHOD OF PRODUCING THEM.

No Drawing.

Application filed December 27, 1920. Serial No. 433,506.

Our invention relates to the manufacture of soluble cellulose-derivatives and products or articles composed of such cellulose derivatives.

5 A common characteristic of most, if not all, the cellulose derivatives such as the ethers and esters, is solubility or uniform miscibility of the cellulose derivatives in or with solvent liquids, and a common characteristic of most if not all, such solvents or liquids of suspension is volatility. Recourse is had to the volatility of the solvent liquids for cellulose derivatives, for the production of many of the articles of manufacture 10 composed of these cellulosic compounds. Of these articles of manufacture, the sheets or films of cellulose ether or cellulose acetate, or the filaments of these cellulose derivatives, may be taken as conspicuous examples.

20 While any such cellulose derivative is capable of being formed into films or filaments by making a solution of the cellulosic material assume the sheet, film, or filament form under conditions favorable to the volatilization of the solvent with retention by the solute of its intended ultimate form, many such cellulose derivatives when left as a residue from solutions, are inflexible, inelastic, brittle, and in such respects mechanically inferior and unsuited to practical uses. Consequently many contrivances in the way of emollients have been resorted to, with more or less success, in order to render 25 cellulosic products better suited to miscellaneous uses.

The object of our invention is to impart to the articles of manufacture composed of cellulose derivatives, such as the ethers and esters of cellulose, the prime quality of flexibility, and the invention is characterized by the association with the cellulose derivative of a substance or substances which are hydroscopic, and which therefore are capable 40 of absorbing into the body composed of the cellulosic compound thus associated with a hydroscopic substance, a uniformly distributed modicum of water, and of retaining the water under all ordinary conditions. 45 Water, thus incorporated into the cellulosic body, enhances the mechanical quality of

flexibility of the article of manufacture composed of the cellulose derivative.

As an example and illustration of our invention: take a cellulose acetate solution in acetone, of such fluidity as to be adapted to the formation of thin films, as by flowing the solution over a glass plate. Mix with the cellulose acetate solution a quantity of zinc chlorid ( $ZnCl_2$ ), from two to ten per cent on the weight of the cellulose acetate dry. The zinc chlorid dissolves through the acetone solution and, when the film is formed in the usual way by volatilization of the acetone, remains uniformly distributed throughout the cellulosic film.

By reason of the presence of zinc chlorid, which is hydroscopic, the film is capable of absorbing water. It will do so gradually if exposed to moist atmosphere; a simple and quick way of supplying the water which the zinc chlorid is capable of absorbing is to wipe the film with a wet cloth. The effect of the water, taken into the film by the action of zinc chlorid may readily be tested by comparing the film made from cellulose acetate alone, and one made from cellulose acetate with zinc chlorid added to it. Take two such test films, of equal thickness, and crease them sharply, back and forth, until the crease in each becomes a line-fracture. With ten per cent zinc chlorid on the weight of dry acetate, in the hydroscopic film, into which water has been fully absorbed, the hydroscopic film has, under test, required from ten to twenty times as many foldings and creasings as the unmodified acetate film, to produce line-fracture.

Another specific illustration of our invention is as follows:—Prepare a solution of ethyl cellulose suitable for film-manufacture, using as a solvent equal parts of ethyl alcohol and acetone. To this solution add from two to ten per cent of zinc chloride (based on the weight of the ethyl cellulose) and form a film from the thus prepared material. We have found that a film made from a solution containing 6% zinc chloride on the weight of the cellulose ether has much greater flexibility than a film of similar thickness, made from a cellulose ether solu-

tion of similar consistency but having no zinc chloride incorporated in it. It required from four to seven times as many foldings to produce line fracture in the film in which zinc chloride was present, as was required to produce line fracture in the film having no zinc chloride in it.

The selection of a hydroscopic substance will be governed by sundry practical considerations; it should not, generally speaking, be capable of chemical reaction with either the cellulose derivative of its solvent, to such extent at least as will deteriorate either, or interfere with the attainment of the final object, in short, the hydroscopic ingredient should be in these relations, substantially inert. Considerations of color which some hydroscopic substances may impart to the final product, will have their weight. The fundamental requisite is, that the substance shall be miscible with the cellulosic solution and residual product, and shall be sufficiently hydroscopic to absorb into the cellulosic body such quantity of water as will serve as a lubricant, emollient, or toughener, to meet the mechanical requirements in each case. Within such limits of proportion as are found practicable the improvement of the physical characteristics of the cellulosic material will be, broadly speaking, proportionate to the amount of hydroscopic material employed.

We claim:

1. A method of modifying organic cellulosic derivatives which consists in permanently incorporating in the organic cellu-

losic derivative a substantially inert hydroscopic substance and causing the same to solidify into a mass and allowing the mass to absorb such water as the hydroscopic 40 substance may absorb and retain.

2. A method of modifying cellulose acetate which consists in permanently incorporating in the cellulose acetate a substantially inert hydroscopic substance and causing the same to solidify into a mass and allowing the mass to absorb such water as the hydroscopic substance may absorb and retain. 45

3. An organic derivative of cellulose, having incorporated therein a substantially inert hydroscopic substance and such water as the hydroscopic substance absorbs and retains. 50

4. The method of modifying cellulose acetate which consists in permanently incorporating zinc chlorid in the body of the cellulose acetate and solidifying the same, subsequently allowing it to acquire such water as the zinc chlorid absorbs and retains. 55

5. Cellulose acetate, having zinc chlorid 60 incorporated in its body and such water as the zinc chlorid absorbs and retains.

6. Cellulose acetate, having from 2 to 10% zinc chloride incorporated therein and such water as the zinc chloride absorbs and retains. 65

Signed by us at New York, N. Y., and Boston, Mass., respectively, this 14th day of December, 1920, and this 16th day of December, 1920.

CAMILLE DREYFUS.  
GEORGE W. MILES.